

May 10, 1932.

McCLEANE BROWN

1,857,620

MANUFACTURE OF HOLLOW METAL BARS

Filed Aug. 9, 1927



McCleane Brown  
By  
O. M. Clarke  
Inventor  
Attorney

## UNITED STATES PATENT OFFICE

MC CLEANE BROWN, OF SEWICKLEY, PENNSYLVANIA

## MANUFACTURE OF HOLLOW METAL BARS

Application filed August 9, 1927. Serial No. 211,710.

My invention refers to the manufacture of metal articles such as stay-bolts, rods, etc., capable of providing resistance, tensile strength and ductility, with a comparatively hard hollow center.

In the manufacture, for instance, of stay-bolts for locomotive fire-boxes or similar uses, it is desirable to provide a small axial perforation, for leakage in case of fracture.

Ordinarily, such perforation is produced by drilling a small hole centrally through the article, and in the case of iron or metals of various kinds, the character as to hardness is usually unvarying throughout the section.

Metal adapted to meet the usual stay-bolt and similar specifications must be sufficiently soft and ductile, with its other qualities, for the necessary ultimate strength, elongation, and reduction of area. The formation of the central perforation by drilling through metal of such character, is difficult because of a lack of sufficient hardness or brittleness, tending to clogging as the drilling proceeds.

This results in great difficulty and rapid wear and breakage of the necessarily small drills used, with an incidental high cost of the product.

In my present invention I utilize in the manufacture of rods, etc., from which stay-bolts or other similar perforated articles are produced, an ingot, slab, bar, or other raw material unit originally made of a pile of metal, as muck bar or the like, as ordinarily utilized in rolling mill practice. Thereafter, the resulting ingot or billet or bar is pierced, in the manner commonly employed in the manufacture of seamless tubing, whereby to effect a complete welding and densification of the metal surrounding the pierced opening, throughout its length.

Thereafter, a piece of tubing coextensive with the length of the bar is inserted in the pierced hole, with as close a fit as can be made, with a filling of sand or other refractory material, and having its ends closed. Thereafter, the pierced bar as thus provided with the tube and its refractory core is re-heated and then reduced by rolling or other suitable means, until reduced to the desired diameter, and with an accompanying proportional re-

duction of the core lining, providing a finally finished central longitudinal comparatively small opening throughout the bar, as hereinafter described.

In the drawings, showing one preferred manner of carrying out my invention:

Fig. 1 is a sectional view in perspective, showing one arrangement of a pile for use in rolling the product;

Fig. 2 is a cross sectional view of the pile after being rolled to the form of a round bar;

Fig. 3 is a partial longitudinal sectional view of the bar thus rolled and illustrating the piercing operation over a mandrel;

Fig. 4 is a cross sectional view of the pierced bar, indicating the dense wall surrounding the central opening;

Fig. 5 is a partial longitudinal sectional view showing the pierced bar provided with the inserted refractory filling tube;

Fig. 6 is a cross sectional view on the line VI-VI of Fig. 5;

Fig. 7 is a view in elevation, partly in section, of a stay-bolt made as one product of the invention;

Fig. 8 is a cross sectional view on the line VIII-VIII of Fig. 7.

Referring to the drawings, I utilize as a base or raw material for the finally rolled rod or bar from which a stay-bolt or other article is made, a pile A, built up in the usual way of rolled bars or other similar elements, scrap, etc.

The arrangement of the individual bars or the like is in any manner suitable to placement in a heating furnace and for the usual reduction to any desirable cross section, as square, hexagon, round, etc.

In utilizing the invention for the making of hollow stay-bolts, the pile is preferably reduced to cylindrical form 2 in cross section, the original separating lines between the individual bars being generally indicated in dotted lines, as at 3. When thus rolled, the resulting bar of suitable diameter is generally similar as to its metallurgical characteristics throughout any cross section, dependent, of course, upon the analysis of the muck bar or other material used in the original pile.

When thus rolled, I then pierce the bar cen-

trally from end to end by the usual or any suitable cross rolling and piercing operation, preferably under the same heat, as indicated in Fig. 3, utilizing a mandrel 4 so as to penetrate the bar 2 from one end to the other, providing the opening 5. In such operation, the middle portion of the bar, surrounding the opening, is subjected to a severe densifying pressure, effecting a complete welding together of the metal, in an annular zone surrounding the opening 5, and with added density, as indicated at 6. In this manner, a strong shell-like cavity is provided, with considerably added resistance as to the strength 15 of the inner wall portion, which is of very considerable advantage in carrying out the later steps of the operation.

Thereafter, a tube 7, of seamless tubing or other suitable pipe form, is inserted within opening 5 from one end to the other of bar 2, as in Fig. 5. The tube 7 is provided with a filling of any suitable refractory material 8, as sand, tightly packed within the tube from one end to the other, the ends being closed in 25 any suitable way, as by swedging them together, or by plugs 9.

As thus provided with the central tube and its refractory core, the bar is then reheated, sufficient to permit of further reduction by 30 rolling, and the diameter of the bar is brought down to suitable dimensions, adapting it to the making of stay-bolts, as shown in Fig. 7. In such reduction, the tube 7 is elongated and reduced in diameter and simultaneously 35 welded to the surrounding bar, during continuous resistance of the refractory 8, so that, in the resulting finished length of bar, there is provided a continuous central opening 10 from one end to the other, and with correspondingly reduced diameter in conformity 40 with the reduced exterior diameter of the finished article.

In carrying out the manufacture of bars in this manner, it is not necessary to subject 45 the refractory core to the same intense heat required in the case of refractory being inserted in a fagot or billet before it is thoroughly welded, or otherwise reinforced, as disclosed herein. The presence of the tubing 7 provides a continuous strong reinforcing lining and holding wall for the refractory, and the tube itself becomes closely impregnated with the main body of the bar and provides the desirable smooth interior. The construction also admits of easy free removal of 55 the refractory after the final rolling operations, either by air or hydraulic pressure, or any other suitable means.

It will be understood, of course, that the 60 relative dimensions of the article, in the original pile form and with a view to the desired eventual or final dimensions of the resulting articles, are within the easy control of the manufacturer, and that any desired cross sectional area or body portion of the pile or

bar may be secured, utilizing suitable metal and in view of its extent of reduction in forging or rolling.

The advantages of the invention will be readily understood and appreciated by all those familiar with the class of hollow stay-bolts and the like, or of any articles requiring the provision of a central smooth continuously open hole.

The original arrangement of the pile itself may be changed or varied within the judgment of the metallurgist or maker, and the invention is in no way restricted to any arrangement of the layers or sections or other specific metallurgical qualities or to any particular or specific shape of the pile or the resulting product in cross section.

I claim:

1. The method of making a hollow center bar or the like from a previously rolled pile of rectangular bars consisting in first forming an axial opening through the rolled bar with surrounding condensation, then inserting within the bar a metal tube containing refractory material, and then reducing the bar and welding it to the tube by pressure.

2. The method of making a hollow center bar or the like from a previously rolled pile of bars arranged in horizontal series consisting in first forming an axial opening through the rolled bar with surrounding condensation, then inserting within the bar a metal tube containing refractory material, and then heating and reducing the bar and tube by external reducing and welding pressure.

3. The method of making a hollow center bar or the like consisting in first assembling a pile of rectangular pieces, rolling the same to cylindrical form, then forming an axial opening through the roller bar with surrounding condensation, then inserting within the bar a metal tube containing refractory material, and then heating and reducing the bar and tube with compensating elongation by external reducing and welding pressure.

4. The method of making a hollow center bar or the like consisting in first reducing a rectangular pile of pieces to cylindrical form, then piercing the bar longitudinally with accompanying condensation of the surrounding metal, then inserting a refractory filled metal tube, and then heating, rolling and welding the bar and tube together.

5. The method of making a hollow center bar or the like consisting in first reducing a rectangular pile of pieces to cylindrical form, then piercing the bar longitudinally with accompanying condensation of the surrounding metal, then inserting a refractory filled metal tube, and then heating, rolling and welding the bar and tube together and removing the refractory from the tube.

6. The method of making a hollow center bar or the like consisting in assembling a pile of rectangular pieces of metal and re-

ducing the same to cylindrical form under heat by rolling, then piercing the center of the resulting bar, then inserting a refractory filled metal tube, and then subjecting 5 the combined bar, tube and refractory core to heat and further rolling and welding.

7. The method of making a hollow center bar or the like consisting in assembling a pile of rectangular pieces of metal and reducing the same to cylindrical form under 10 heat by rolling, then piercing the center of the resulting bar, then inserting a refractory filled tube, and then subjecting the combined bar, tube and refractory core to heat 15 and further rolling and welding with final removal of the refractory.

8. A hollow metal bar consisting of a main outer integral densified body portion formed from a variously distorted elemental rolled 20 cylindrical blank having a central metal tube incorporated by welding with the surrounding densified inner portion of the outer body portion.

9. A hollow metal bar consisting of a main outer integral densified body portion formed from a variously distorted elemental rolled cylindrical blank having a central metal tube incorporated by welding with the surrounding 25 densified inner portion of the outer body portion and welded thereto.

In testimony whereof I hereunto affix my signature.

McCLEANE BROWN.

25

40

45

50

55

60

65

**CERTIFICATE OF CORRECTION.**

**Patent No. 1,857,620.**

**May 10, 1932.**

**McCLEANE BROWN.**

**It is hereby certified that error appears in the printed specification of the above numbered patent requiring correction as follows: Page 2, line 105, claim 3, for the word "roller" read rolled; and that the said Letters Patent should be read with this correction therein that the same may conform to the record of the case in the Patent Office.**

**Signed and sealed this 12th day of July, A. D. 1932.**

**(Seal)**

**M. J. Moore,  
Acting Commissioner of Patents.**